

F. L. ANTISELL.  
PROCESS FOR TREATING COPPER.  
APPLICATION FILED NOV. 1, 1912.

1,204,927.

Patented Nov. 14, 1916.



WITNESSES

INVENTOR  
*F. L. Antisell*  
BY  
*W. A. Meyrath*  
ATTORNEY

# UNITED STATES PATENT OFFICE.

FRANK L. ANTISELL, OF PERTH AMBOY, NEW JERSEY.

## PROCESS FOR TREATING COPPER.

1,204,927.

Specification of Letters Patent. Patented Nov. 14, 1916.

Application filed November 1, 1912. Serial No. 728,984.

To all whom it may concern:

Be it known that I, FRANK LINDEN ANTISELL, a citizen of the United States, and a resident of Perth Amboy, county of Middlesex, State of New Jersey, have invented certain new and useful Improvements in Processes for Treating Copper, of which the following is a specification.

My invention relates to the process of and 10 furnace for treating copper.

The objects of the invention will appear from the hereinafter description.

Before describing my improvements it may be well to briefly outline the prevailing 15 process and accepted principles relating to the refining of what is known as cathode copper which results from the electrolytic refining of copper.

Copper in cathode form will run in conductivity (Matthissen standard) as high as 20 102 per cent., and the copper contents of said cathode will be as high as 99.97 per cent.

By the present process of melting the cathode copper into proper shape for drawing 25 into wire or rolling into plates or cakes both the electric conductivity and copper contents are lowered by reason of the melting down being performed in an ordinary reverberatory furnace which is generally heated by 30 coal, and the flame being only under partial control at times, the character of the flame constituting changes from an oxidizing flame to a reducing flame. While each kind of flame is valuable at the proper time in the 35 melting down, at other times such a flame is detrimental. The tendency of the oxidizing flame is to form copper oxide as well as oxides of the other impurities that may be present in the molten copper, such as iron, zinc, etc., 40 which are skimmed off with the oxide slag. The sulfur which has been dissolved during the process of melting passes off as sulfur dioxide and part of the arsenic and antimony passes off as lower oxides. This oxidizing is 45 generally facilitated by "flapping" or blowing air in the molten copper. After this the molten copper is subjected to the step in the art of what is known as "poling" where charcoal is spread over the surface of the

molten copper and a stick of green wood is 50 forced under the surface of the copper which reduces the oxides of copper and to some extent the oxid impurities in the molten copper. This step is carried on until the oxides of copper are reduced to some  $\frac{3}{10}$  or  $\frac{4}{10}$  of 55 1 per cent. If the step of poling is carried to completely reduce the higher oxides, that is, the oxides of arsenic and antimony which are present, they are reduced to a metallic state and alloy with the copper, reducing its 60 conductivity. In addition to reducing said oxides the copper absorbs the gases from the green wood and "overpoles" or "spues" are produced which give the copper a high "pitch" which makes it brittle and lower in 65 conductivity. In this condition reflapping and repoling of the molten copper is necessary. It is therefore evident that it is desirable to reduce the oxides of copper to the lowest per cent. and still not affect the other 70 oxides present, such as arsenic and antimony.

Attempts have been made by others to melt copper without contaminating it by the flame, which contamination is proportionate to the time the flame plays on the copper. 75 One of the various attempts to obtain this result has been to melt the cathode copper under cover or blanket of suitable character in the nature of non-metallic salt of which boron trioxide is one, which will prevent the 80 air and gases coming into contact with the copper as it melts. This attempt has been found to be unsatisfactory in practice, however, owing to the increased amount of heat necessary to melt the copper under the 85 blanket. Furthermore, the intense heat necessary to melt the copper under the blanket causes the blanket to flux the silica in the side of the furnace with its apparent disadvantages. The blanket itself volatilizes and is carried off up the stack under the intense heat, at a great loss. I have overcome these objections by preheating the copper and then melting it in a proper furnace and conveying or transferring the melted 90 copper from said furnace in its molten condition under a blanket which covers the surface of the copper and prevents its contact

with air, gas or other contaminating elements. While I prefer to preheat the copper, yet it is not necessary.

My process may be carried out by different apparatus, but in the accompanying drawing I have shown two types of apparatus especially adapted for my purpose.

This application is a continuation in part of my prior application Serial No. 10 608,935, filed February 6, 1911.

Referring to the drawing: Figure 1 is a section of a melting furnace and a purifying furnace showing the relative arrangement and the connection between the same. Fig. 15 2 is a sectional view of the preferred form of treating furnace. Fig. 3 is a section on line 3 of Fig. 2.

In the drawing the part marked A represents the melting furnace. 10 is the crucible 20 thereof.

11 is the superstructure for preheating the charge.

12 represents the oil burners communicating with the furnace to feed the oil fuel 25 thereto.

13 is a tap hole at the bottom of the furnace leading to the spout 14.

B is a reheating or treating furnace which has a closed chamber 15 having an opening 30 16 in the top thereof in communication with the spout 14. This chamber has a tap hole 17 communicating with the spout 18. The chamber 15 contains preferably carbon in a finely divided form or it may contain boron-trioxide mixed with carbon also preferably in a finely divided form. Under the chamber 35 15 is a combustion chamber 19 heated by liquid fuel passing through the burner 20.

In operation the charge W as fed into the 40 furnace A is heated and reduced to a molten state by the fuel passing through the burners 12. It is to be understood, of course, that the action of the flames in the open air causes more or less oxidation of the copper 45 and the impurities contained therein. The products of combustion pass up through the preheated structure 11 and preheat the charge W. The molten copper passes through the tap hole 13, through the spout 50 14, through the opening 16, into the chamber 15, through the carbon or boron-trioxide and carbon and rises in the chamber and causes said carbon or carbon and boron-trioxide to float upon the molten copper in the chamber B, the said carbon or boron-trioxide and carbon forming a cover or blanket C over the molten metal. This molten copper is drawn from chamber 55 15, through the tap hole 17 into the spout 18, where it is conveyed to proper molds not shown. The molten metal in the chamber 15 is kept in its proper heated condition by the burning of the fuel in the combustion chamber 19.

Referring to the construction shown by

Figs. 2 and 3, D is a furnace divided into 65 two compartments 21 and 22 by the partition 23, leaving a passageway 24 between the two compartments. The furnace is heated by a supply of liquid fuel through the burner 25. 26 is a stack communicating 70 with the chamber 22. The bottom of the stack is inclined as shown at 27, down which the charge W' is passed through an opening 28. C' represents carbon preferably in a finely divided form or boron-trioxide mixed 75 with carbon. 29 is a tap hole closed by a plug of clay 30 in the usual manner. 31 is an opening in the chamber 21 above the blanket.

As shown in the drawing, the burners 12 80 and the burner 25 are supplied with valves for the purpose of so regulating the same as to produce an oxidizing flame.

In operation the furnace is heated by the fuel fed to the burner 25, the products of 85 combustion passing up through the stack 26. The charge W' is fed through the opening 28, down the incline 27, where it is preheated by the products of combustion. The charge falls down into the chamber 22, where it is 90 reduced to a molten state. The molten charge passes through the passageway 24 and underneath the carbon C' or boron-trioxide and carbon in the chamber 21, which forms a cover or blanket over the molten 95 metal in said chamber. The molten metal is drawn from the tap hole 29 by withdrawing the plug 30, when desired.

As indicated in the drawing, the melting down of the charge is accomplished by 100 means of an oil fuel furnace which I term a combination melting and purifying furnace, the melting part being in the nature of a reheating furnace where the flame after being thoroughly consumed in the combustion 105 chamber passes over a relatively small bath of copper and then ascends through the stack or cupola of the furnace meeting the incoming charge of cathode sheets which are thereby heated to nearly a fusing temperature, the hearth or crucible adding little more than the heat of fusion to the already hot copper sheets. This operation is carried on so rapidly and efficiently that the copper has time to absorb but a small percentage of 11 impurities which otherwise would have been absorbed had the metal been melted down in an ordinary furnace, where possibly 200,000 to 400,000 lbs. of copper are piled in the open hearth and melted down during a 12 period of five or six hours to a flat condition; that is to say, there is a small layer of molten copper over the mass of unmelted copper on the bottom of the furnace.

To melt the copper off the bottom, it is 12 necessary to fire the furnace hard for several hours, which operation during this period cannot be termed "fusing" in the strict

meaning of the term, as it is rather one of "dissolving" where the upper layer of copper is kept in a molten condition and the copper submerged is liquefied by the contact of the molten copper.

As the laws of efficiency of heating surfaces are based fundamentally upon the difference in degrees of temperature between the absorbing medium and the heat emanating medium, and as molten copper has a temperature of 2000° F., in round numbers, and assuming that the flame over the bath has a temperature of 2500° (a very usual observed temperature), there is only some 10 20 per cent. of the heat that is efficient for melting the copper, the 80 per cent. of the heat passing out of the stack at 2000°. But by preheating the copper the gases pass from the furnace at a much lower temperature, resulting in both an economy of fuel and time for melting.

The principal advantage gained by the improved process is in decreasing the amount of foreign substances absorbed by 25 the copper, by reason of the time interval reduced in minutes in place of hours for melting, and immediately after melting, running into a separate compartment from the melting compartment where it is refined 30 by means of the boron-trioxide and carbon or carbon itself, which acts as a reducing agent. It is therefore evident that by charging copper in the preheating chamber I am able to melt continuously, transferring 35 the same to the purifying chamber and casting either continuously or intermittently as I desire.

I prefer to build my furnace partitioned as shown by Figs. 2 and 3 of the drawing 40 and leave a large communicating port between the partition and bottom of the furnace, and depend upon the thermal conductivity of the copper for keeping the metal in the reducing compartment at a suitable temperature for refining. This construction would also offer some advantage due to the osmotic pressure which would be exerted between refined and unrefined copper tending 45 to keep it in a nearly uniform condition throughout the melting compartment.

In carrying out my process, the pre-heating is effected by means of a heat which is not sufficient to melt the copper, and therefore the step of pre-heating in my process is 50 clearly distinguishable from the initial action of the melting heat upon the copper. The pre-heating is never accomplished by the action of the melting heat, but is always accomplished by a heat which is always less 55 than the melting heat and insufficient to accomplish the melting of the copper. It is in this sense that I have used the word "pre-heating" in the specification and claims.

Having now described my invention,

what I claim as new and desire to secure by Letters Patent is:

1. The process of refining copper which consists in simultaneously melting and oxidizing copper and then passing the oxidized melted copper through a material containing carbon.

2. The process of refining copper which consists in simultaneously melting and oxidizing copper and then passing the oxidized melted copper through carbon.

3. The process of refining copper which consists in simultaneously melting and oxidizing copper and then passing the oxidized melted copper under a material containing carbon.

4. The process of refining copper which consists in simultaneously melting and oxidizing copper and then passing the oxidized melted copper under a reducing agent.

5. The process of refining copper which consists in simultaneously melting and oxidizing copper and conducting the oxidized melted copper under a blanket of a material containing carbon.

6. The process of refining copper which comprises exposing the same to the heat of a furnace and its gases until reduced to a molten condition, then removing the copper from exposure to said gases and into contact with carbon sufficient to purify said copper.

7. The process of refining copper consisting in exposing the same to the heat of a furnace and its gases until reduced to a molten condition, then removing the copper from exposure to said gases, and passing said copper through and under a protective flux and in contact with carbon.

8. The process of treating copper consisting in exposing the same to the heat of a furnace and its gases until reduced to a molten condition, removing the copper from exposure to said gases by passing said copper through and under a protecting flux of boron trioxide containing carbon, retaining said copper in contact with the carbon, and then flowing said copper to a ladle or mold while out of contact with furnace gases.

9. The process of purifying copper associated with sulfur which consists in continuously causing copper to become molten thereby introducing therein copper oxid, and then continuously bringing the molten mass in contact with carbon until the greater portion of the copper oxid is reduced.

10. The process of treating copper which consists in preheating and oxidizing copper in a chamber by means of highly heated products of combustion, removing the mass and subjecting it to a reducing medium.

11. The process of treating copper which consists in continuously melting and oxidizing copper, continuously removing the cop-

- per, and subjecting the copper to the action of a reducing medium.
12. The process of treating copper which consists in continuously melting and oxidizing copper, and continuously reducing the said melted and oxidized copper.
13. The process of purifying copper associated with sulfur which consists in continuously causing the copper to become molten thereby introducing therein copper oxide and then bringing the molten mass in contact with carbon until the greater portion of the copper oxide is reduced.
14. The process of refining copper which consists in first melting and oxidizing the copper and then subjecting the melted oxidized mass to the action of a reducing agent and to the action of an anhydrous body to separate oxide therefrom.
- 20 15. The process of refining copper which consists in first melting and oxidizing the copper and then subjecting it to the action of a reducing agent and a dissolving agent.
- 25 16. The process of refining copper which consists in first melting and oxidizing the copper and then subjecting it to the action of a dissolving agent and to the action of a reducing agent.
- 30 17. The process of refining copper which consists in first melting and oxidizing the copper and then subjecting the melted oxidized mass to the action of dissolving and reducing agents.
- 35 18. The process of refining copper which consists in first melting and oxidizing the copper and then subjecting it to the action of dissolving and reducing agents to coact with the oxygen of the copper.
- 40 19. The process of treating copper, which consists in melting copper in a chamber by means of the highly heated products of combustion of a fluid fuel burner, removing the copper to a point exterior of said chamber, and delivering the copper to a reducing medium.
- 45 20. The process of refining copper which consists in melting and oxidizing copper and conducting the molten copper under a blanket of carbon.
- 50 21. The process of refining copper which consists in preheating copper, heating the preheated copper until it becomes molten, and conducting the molten copper through carbon.
- 55 22. The process of refining copper which consists in preheating the copper, heating the preheated copper until it becomes molten, and conducting the molten copper through and under a blanket of carbon.
- 60 23. The process of refining copper which consists in preheating copper, melting the preheated copper in a furnace, and conducting or conveying the molten copper to a chamber containing carbon.
24. The process of refining copper by preheating to a high temperature outside of the melting zone, melting the preheated copper as rapidly as possible, and transferring the melted copper to a refining chamber containing carbon.
- 70 25. The process of treating copper which consists in preheating copper, heating the preheated copper until it becomes molten, and refining the molten copper by bringing it into contact with carbon.
- 75 26. The process of refining copper which consists in first preheating and then melting copper in a melting compartment, running the molten copper into a separate compartment, and refining the copper in the latter compartment by carbon.
- 80 27. The process of refining copper which consists in charging the copper into a chamber, continuously melting down the copper, transferring the same to a purifying chamber containing carbon, and casting the copper from said purifying chamber.
- 85 28. The process of treating copper which consists in continuously charging the copper into a heating chamber, treating the copper in the heating chamber to an oil fuel flame until it becomes molten, subjecting the incoming charge of copper to the outgoing flame, conducting the molten copper to a separate chamber or compartment containing carbon, and purifying the copper in the latter chamber.
- 90 29. The process of refining copper which consists in preheating the copper, melting the preheated copper, carrying the melted copper out of contact with contaminating elements, and refining the same by bringing it into contact with the carbon.
- 95 30. The process of refining copper which consists in exposing the copper to the heat of a furnace and gases until reduced to a molten condition, then removing the copper from exposure to said gases and into intimate contact with carbon to purify the copper.
- 100 31. The process of refining copper which consists in exposing copper to the heat of a furnace and its gases until reduced to a molten condition, removing the molten copper from exposure to said gases and into intimate contact with carbon to purify the copper, and then conducting the copper to a mold out of contact with said furnace gases.
- 110 32. The process of refining copper which consists in reducing copper to a molten condition by heat, removing the copper from exposure to the source of heat, bringing the copper into intimate contact with carbon until the greater portion of the copper oxide is reduced, and then conducting the copper to a mold and out of contact with the furnace gases.
- 120 125

33. The process of refining copper which consists in preheating copper, subjecting the preheated copper to an oil fuel flame until it becomes molten, transferring the melted copper out of contact with the flame and the gases thereof, and bringing it into contact with carbon.

In witness whereof I have hereunto set

my hand, at the city, county, and State of New York, this twenty-second day of October, 1912.

FRANK L. ANTISELL.

In presence of—

I. RICHARDS,  
A. C. O'CONNELL.